

Jan. 30, 1934.

J. C. SIEGLE

1,945,087

METHOD OF TREATING CAST HOLLOW INGOTS

Filed Jan. 29, 1932



Fig. 2.

INVENTOR  
Jacob C. Siegle.

BY Henry S. Hellert  
ATTORNEYS

WITNESS

F. J. Hartman.

## UNITED STATES PATENT OFFICE

1,945,087

METHOD OF TREATING CAST HOLLOW  
INGOTSJacob C. Siegle, Youngstown, Ohio, assignor to  
The Youngstown Sheet and Tube Company,  
Youngstown, Ohio, a corporation of Ohio

Application January 29, 1932. Serial No. 589,563

8 Claims. (Cl. 29—160.4)

This invention relates to the treatment of hollow cylindrical ferrous bodies having irregularities and impurities in their inner surfaces and is particularly directed to a method of treating 5 centrifugally cast hollow ingots to smooth up their said surfaces and/or remove segregations of foreign material lying adjacent thereto.

When hollow ingots are cast centrifugally, the molten metal is poured into a rapidly rotating 10 mold and the rotation of the mold continued until the metal is substantially solidified. As the centrifugal force acting upon the molten metal urges it very strongly against the walls of the mold, material of less density than the 15 metal and contained therein is carried toward the center and may ultimately reach the inner surface of the ingot, wherein the interior surface of the finished ingot is usually quite rough. When ingots or pipes formed in this manner are 20 used as made, without further working of the metal; for example, when they are filled with concrete to form pilings, or the like, the roughened interior so produced may be of appreciable value in retaining the concrete in the pipe, but 25 when it is desired to work the ingot into relatively thin walled pipes and tubes this internal roughness is a distinct disadvantage and coupled with the presence of the segregations tends 30 to the production of defects in the finished articles.

The principal object of the present invention, therefore, is to provide a method of treating hollow ingots whereby roughness of their interior surfaces and segregations of foreign matter 35 incorporated therein may be readily removed and relatively smooth interior surfaces of substantially pure metal may be produced instead.

A further object of the invention is to provide a method of treatment of ferrous bodies of the 40 class described in the course of which the material forming the inner surfaces thereof is locally oxidized and thereby converted into a relatively brittle scale, the subsequent removal of which leaves a smooth surface on the interior of the 45 body.

Another object of the invention is to provide 50 apparatus suitable for the performance of the said method and comprising in combination with a heating furnace in which the ingots are brought to desired working temperature, means 55 operative to introduce an oxidizing fluid into the interior of the ingots as they pass successively through the furnace to thereby convert the inner surface metal and any foreign segregations included therein into oxides which may be readily

cracked or broken away during subsequent attenuation of the ingot or other working thereof in a suitable rolling mill or other apparatus.

Other purposes, objects and advantages of the invention will hereinafter more fully appear or will be understood from the following description of a preferred manner of performing the method by means of the said apparatus, reference being had to the accompanying drawing in which Fig. 1 is a diagrammatic horizontal section of a heating furnace suitably equipped for the practice of the method with a plurality of ingots disposed in its interior, and Fig. 2 is a diagrammatic fragmentary side elevation of a skew roll piercing mill or like apparatus employed 60 for working the ingot and breaking off the internal scale after the furnace treatment, a portion of an ingot in its passage through the mill being shown in vertical section.

The furnace F shown in Fig. 1 may be of any 65 usual type adapted for heating the ingots to proper working temperature, its walls being formed of refractory material such as fire brick or the like. Charging skids C or other suitable means may be disposed adjacent the charging 70 port P at one end of the furnace to facilitate introduction of the ingots, and spaced skids S may be arranged inside the furnace to support the ingots I as they are moved gradually and 75 consecutively through the latter while they are being heated. The ingot discharging apparatus at the opposite end of the furnace comprises a 80 pusher R which may be projected through a port P' into the furnace and successively into engagement with the adjacent end of each ingot 85 as it reaches working temperature to thereby force it axially outwardly through a port P'' onto a conveyor D or other receiving apparatus 90 from which it may be carried by a crane or other suitable conveying means to the apparatus provided for the next ensuing operation. The 95 several ports are normally closed by suitable doors (not shown) in the ordinary way.

It will be understood that the traverse of the 100 ingots through the furnace usually, and in accordance with my invention, progresses at a rate sufficiently slow to enable them to absorb the requisite amount of heat from heated gases supplied to the furnace by any usual means (not shown) to raise them to the desired working temperature and that the ingots are discharged one at a time through the port P'' when they have reached that temperature, conveying means of any suitable type being usually provided for 105 moving the ingots along the skids S.

110

According to my invention I extend through the walls of the furnace, preferably near its exit end and thus relatively close to the conveyor D, one or more nozzles 1, two being generally preferred, which respectively project into the furnace and terminate in jets 2 at longitudinally spaced points adjacent the path of travel of the ingots when disposed on the skids S and substantially in the plane of their axes. Each nozzle has a longitudinal passage in its interior and is interconnected with a supply pipe or manifold 3, through a valve 4, from which compressed air, oxygen, or other gaseous oxidizing fluid from any suitable source (not shown) is supplied. If desired, a larger number of nozzles than two may be provided and arranged in parallel relation at suitably spaced points and all connected to the manifold supply pipe 3, while additional like nozzles 1' may be respectively interconnected with another manifold supply pipe 3' through valves 4' on the opposite side of the furnace as indicated in dotted lines in Fig. 1. Each of the nozzles as controlled by its valve is thus capable of projecting a quantity of gaseous, oxidizing fluid into the interior of the ingot respectively disposed in alignment therewith on the skids S when the nozzle valve is opened.

In the practice of the method of my invention by means of an apparatus of the character to which I have referred, the cast hollow ingots are moved successively through the furnace F until they come into alignment with the nozzles which are then so operated as to inject air, oxygen or other gaseous oxidizing fluid into the bores of the ingots, preferably as they approach the desired working temperature. Thus, the usual heating operation required to raise the ingots to that temperature is in no way interfered with or modified, the oxidizing medium being preferably introduced, as stated, as the end of the heating period for each ingot is approached. However, in the preferred practice of the invention, the quantity of the oxidizing fluid utilized is such that substantially the entire amount introduced is retained within the ingot and the preferably neutral or slightly reducing character of the atmosphere within the main chamber of the furnace therefore remains substantially unaffected while the atmosphere within the individual ingots is made highly oxidizing in character.

After the oxidizing fluid is introduced into the interior of the heated ingots through the jets 2 at the inner ends of the nozzles 1 by manual or automatic opening of the valves 4 and 4' when the ingots are in alignment with the nozzles, the oxidation of the material forming the inner walls of the ingots proceeds at a fairly rapid rate due to its relatively high temperature so that a relatively thick or heavy scale composed of metallic oxides and of any other impurities which may be carried thereby in the form of segregations is soon produced within the ingot. Moreover, as the metal in the interior of the centrifugally cast ingots frequently solidifies in small projections, it is apparent that the latter, if present, will also be substantially oxidized into scale and that the metal underneath the scale will consequently be relatively smooth after the scale has been removed. Scale of this character is extremely hard but is relatively brittle and may be readily cracked loose from the unoxidized metal of the ingot when the latter is attenuated or otherwise worked by suitable means during the subsequent operations customarily in-

cident to the formation of pipes and tubes from hollow ingots.

Thus, for example, removal of the scale may be readily effected by passing the ingot through a mill of the character of that indicated in Fig. 2 and thus comprising a pair of diagonal or skew rolls 5 of suitable shape and a mandrel or piercing head 6 disposed therebetween. It is believed the operation of this apparatus will be readily understood as it is not substantially different from that of the ordinary diagonal or cross roll piercing mill, the working of the metal as the ingot passes through the mill serving to break the scale loose from the inner wall of the ingot from which it can then be readily removed as a loose and rather finely divided deposit by means of a blast of air or in any other suitable way. In the diagonal rolling referred to it is, of course, not necessary to permanently change the form of the ingot by attenuation of the metal in order to break the scale loose therefrom but as such attenuation is generally effected on ingots of this character in accordance with the methods of operation now in use for forming pipes or tubes therefrom, the scale removal will usually be carried out coincidentally with and as a part of a rolling operation primarily designed to elongate the ingot rather than as a separate step directed to the removal of the scale alone.

I have found that ingots which have been treated as hereinabove described are substantially free from undesirable projections or roughness on their interior surfaces and from segregations of foreign material and/or other impurities adjacent thereto, either or both of which, as is well known in the industry, frequently cause serious defects in the finished tubes or pipes if not removed before the formation thereof from an ingot. Additionally, by suitably controlling the amount of oxidizing fluid introduced into the ingots in the furnace, the oxidation of their exterior surfaces is not materially increased beyond the normal amount which occurs under ordinary heating conditions, since, desirably, only sufficient oxidizing fluid is admitted to effect a rather heavy oxidation of the interior surface of each ingot without substantially affecting the preferably neutral or slightly reducing character of the atmosphere generally in the furnace chamber.

Thus by my invention, I am enabled to produce smooth pipes and tubes of high quality free from many of the defects which occur in pipes and tubes made from centrifugally cast hollow ingots in accordance with the methods now in use and by means of apparatus now employed for such purposes, but without appreciably increasing manufacturing costs, since the apparatus employed is of relatively simple and inexpensive character and requires but little attention for its proper operation.

While I have herein described my invention with particular reference to the preferred manner of practising my improved method by means of apparatus of the character herein disclosed, it will be understood that a heating furnace of form or type other than that to which I have referred may be employed, and that changes in the design and arrangement of other parts of the apparatus and/or in the specific mode of operation thereof in carrying out the method may be made, if desired, without departing from the spirit and scope of the invention as defined in the appended claims.

Having thus described my invention, I claim

- and desire to protect by Letters Patent of the United States:
1. The method of preparing a hollow ingot for subsequent working which comprises the steps of heating the ingot to working temperature and during such heating introducing into the interior thereof gaseous oxidizing fluid to form a scale, and thereafter working the ingot to free the scale from the bore. 5
2. The method of preparing a hollow ingot for subsequent working which comprises the steps of heating the ingot to a predetermined temperature in a substantially non-oxidizing atmosphere and prior to the attainment of that temperature injecting into the bore of the ingot a gaseous fluid adapted to oxidize the metal surrounding the bore to thereby form a heavy scale on the wall thereof. 10
3. In a method of treating hollow ingots, the step of injecting a gaseous oxidizing fluid into the bore of each ingot while the ingot is at a sufficient temperature to react relatively rapidly with said fluid to thereby form a scale, and thereafter working the ingot to free the scale from the bore. 15
4. The method of treating a hollow centrifugally cast ingot which comprises the steps of positively effecting oxidization of its interior surface only so as to form a scale thereon and thereafter working the ingot to free the scale from said surface. 20
5. The method of treating hollow centrifugally cast ingots to remove internal roughness and segregations of impurities which comprises the steps of successively heating the ingots in a heating furnace to raise them to a predetermined working temperature, injecting into the bore of each ingot a gaseous medium adapted to oxidize the metal surrounding said bore, then removing the ingot from the furnace, and finally working the metal 25
- thereof to crack off the scale formed in the bore by said oxidation. 30
6. The method of treating hollow centrifugally cast ingots to remove internal roughness and segregations of impurities which comprises the steps of consecutively heating the ingots in a heating chamber containing substantially non-oxidizing atmosphere to thereby raise the ingots to a predetermined working temperature, injecting into the bore of each ingot while in the chamber a gaseous medium adapted to effect relatively rapid oxidation of the metal surrounding said bore, removing the ingots consecutively from the furnace, and finally working the metal thereof in such manner as to break off the scale formed in the ingot bores by said oxidation. 35
7. The method of treating a centrifugally cast hollow ingot to remove internal roughness and impurity segregations which comprises the steps of heating the ingot to a predetermined working temperature in a substantially non-oxidizing atmosphere and, while in said atmosphere, creating a strongly oxidizing atmosphere in the bore of the ingot to thereby oxidize the metal surrounding the bore and form a heavy scale, then removing the ingot from the heating zone, and finally working the metal of the ingot so as to crack said scale away from the wall of the ingot bore. 40
8. The method of treating a centrifugally cast hollow ingot to remove internal roughness and impurity segregations which comprises the steps of heating the ingot to a predetermined temperature, positively creating a strongly oxidizing atmosphere in the bore of the hot ingot to thereby oxidize the metal surrounding the bore and form a heavy scale, and then working the metal of the ingot so as to crack said scale away from the body of the ingot. 45
- JACOB C. SIEGLE. 50
- 120
- 125
- 130
- 135
- 140
- 145
- 150